

Patented Sept. 5, 1922.

1,427,970

# UNITED STATES PATENT OFFICE.

GEORGE W. PLEIS, SR., AND GEORGE W. PLEIS, JR., OF PHILADELPHIA, PENNSYLVANIA.

## SECONDARY BATTERIES.

No Drawing.

Application filed June 6, 1921. Serial No. 476,003.

To all whom it may concern:

Be it known that we, George W. Pleis, Sr., and George W. Pleis, Jr., citizens of the United States, and residing at Philadelphia, in the county of Philadelphia and State of Pennsylvania, have invented certain new and useful Improvements in Secondary Batteries, of which the following is a specification.

10. This invention relates to secondary batteries, and more particularly to the electrodes of such batteries.

An object of my invention is to produce a battery which will withstand rough treatment with a minimum of loss of active material from the electrodes.

Another object is to produce an electrode for such batteries that will charge and discharge more rapidly than is customary, 20 without deterioration.

Another object is to produce a plate which may be converted into either a positive or a negative electrode, by the forming process, and be highly durable in either condition.

25. Other objects will appear on reading the specification.

The electrodes are made as follows:

A modern standard type of grid of any ordinary construction is selected, and a 30 paste, described below, is thoroughly worked into it, preferably by hand labor. The paste is made as follows:

Yellow accumulator oxide (litharge) 60 lbs. to 70 lbs.  
35 Red accumulator oxide (red lead) 40 lbs. to 30 lbs.  
Talc powder 5 lbs. to 10 lbs.  
Lamp black 1 lbs. to 2 lbs.

40. The above powders are thoroughly mixed in a tumbling machine, uniformity in composition being essential. A quantity of the dry mixture, about one hundred pounds, is now put on a glass or other acid proof plate, 45 and shaped into a ring, into the center of which is then poured slowly thirty five hundred cubic centimeters to four thousand cubic centimeters of "purified granular ammonium sulphate" solution, of specific gravity 1.100 to 1.140, mixing the two thoroughly with a wood paddle. After standing for about five minutes, or long enough so that the mixture does not become "shocked", (in other words, after standing for about five

50 minutes the chemical action that takes place prevents subsequent disintegration of "set"

paste), a similar quantity of the ammonium sulphate solution, making seven thousand to eight thousand cubic centimeters in all, is added; and thoroughly incorporated in the mass. The finished paste is now ready to be worked into the grids.

The ammonium sulphate solution is made by dissolving what is known in the trade as "ammonium sulphate, granular purified" 60 in distilled water, until it reaches a specific gravity of 1.100 to 1.140. The solution should be covered to protect it from dust, etc., and allowed to stand at least ten hours before using.

70. The plate is filled upon a grid block, or support, consisting of a wood block upon which is a beveled heavy glass plate, the top being the size of the grid to be filled. Over the glass is secured a layer of absorbing material such as cloth, linen, canvas, heavy paper, fibre, etc., the fabric being stretched tightly and secured on all sides to the wood block by cleats, etc. A grid is now placed on the covered block, and the above described paste thoroughly worked in preferably by hand labor, using a wood rammer, particular care being taken that all of the recesses and corners within the grid are filled and compacted to a substantially uniform density. It is important that all 80 spaces be filled with the paste, and that all of the plates be compacted to the same density. The pasted grids are now slid sideways off of the grid block and placed upright in frames and left to dry for a period varying from fifteen to thirty minutes, varying with the size, thickness, etc., of the grid, also of the weather. Artificial drying may be resorted to if desired, in which case the time 85 of drying will depend upon the factors of the drying process. After the drying period has passed, the plates are slowly immersed in a sulphuric acid solution, specific gravity 1.100 to 1.200, for from nine to sixteen hours, varying with the size of the plate. After this period of immersion has 90 passed, the plates are taken out and allowed to dry. They are then ready for assembling for the "forming" process.

100. The sulphuric acid of 1.100 to 1.200 specific gravity consists of chemically pure acid and distilled water, and after mixing should be allowed to stand for at least twenty four hours before using.

110. All of the electrodes are made by the above method, there are no special compositions

for positive plates, and different compositions for negative plates.

- A number of plates are now assembled in a group, and another assembled group interlaced therewith, the two groups then immersed in battery acid and charged and discharged through generally two cycles, and then given a final charge. They now are in the condition of positives and negatives.
- 10 The number of charging cycles may be increased if desired. After forming, a suitable number of the positives are united by a connecting yoke, and also a suitable number of negatives, to constitute a battery.
- 15 After assembling, they are properly sealed in a cell, charged, and the battery is ready for use.

We claim:

1. A secondary battery electrode having active material containing lead oxids, talc, and lamp black.
2. A secondary battery electrode having active material containing 90 to 95% lead oxids, from 9 to 4 per cent of talc, and, 25 about one per cent of lamp black.
3. The method of making a secondary battery electrode which comprises mixing lead oxids, talc, and lamp black, moistening the mix with ammonium sulphate solution 30 to form a paste, pressing the paste into a grid, and soaking the grid in sulphuric acid solution.
4. The method of making a secondary battery electrode which comprises mixing lead oxids, talc, and lamp black, moistening the powdered mix with ammonium sul-

phate solution of 1.100 to 1.140 sp. g. to form 40 a paste, pressing the paste into a grid, and soaking the grid in sulphuric acid of 1.100 to 1.200 sp. g.

5. The method of making a secondary battery electrode, which comprises mixing lead oxids, talc, and lamp black, moistening the powdered mix with ammonium sulphate solution of 1.100 to 1.140 sp. g., allowing to stand for about five minutes, adding a further quantity of ammonium sulphate solution and mixing, pressing the paste into a grid, allowing to stand less than 30 minutes, depending on the size of the grid, and then immersing in sulphuric acid solution for 50 from 9 to 16 hours.

6. The method of making a secondary battery electrode, which comprises mixing lead oxids, talc, and lamp black, moistening the powdered mix with ammonium sulphate solution of 1.100 to 1.140 sp. g. allowing 60 to stand for about five minutes, adding a further quantity of ammonium sulphate solution and mixing, pressing the paste into a grid, allowing to stand less than 30 minutes depending on the size of the grid, then 65 immersing in sulphuric acid solution for from 9 to 16 hours, then subjecting to a forming process, by connecting as a positive to form a positive plate, or as a negative to form a negative plate.

In testimony whereof we hereby affix our signatures.

GEORGE W. PLEIS, Sr.  
GEORGE W. PLEIS, Jr.